

## UNITED STATES PATENT OFFICE

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE

## ACID PROCESS OF FIBER LIBERATION

No Drawing.

Application filed October 26, 1929. Serial No. 402,797.

This invention relates to the production from wood or other raw cellulosic materials of a high grade chemical pulp characterized not only by excellent physical characteristics, including strength and tear resistance, but also by easy bleachability, so that it may be converted into a white product suitable for high grade papers, with low bleach consumption and without substantial injury to its physical or chemical characteristics.

The so-called acid sulphite process of fiber liberation is employed for the production of light-colored pulps which are bleachable to the whiteness desired in high grade papers, without excessive degradation of the cellulose or injury to the fibers. In practising this process of fiber liberation, chipped wood or other raw cellulosic material is cooked under conditions of high temperature and pressure in a liquor consisting of a sulphurous acid solution of a sulphite of calcium, magnesium, sodium, or the like, containing about 4% to 7% free SO<sub>2</sub>, which is gradually released from the liquor during the cooking operation, while the temperature of cooking is increased.

In accordance with the process of the present invention, fiber liberation is completed in a liquor of lower combined SO<sub>2</sub> content than that of the fresh liquor in which cooking is started, as I have found that such a process makes possible the production of a pulp of improved characteristics, including higher strength and tear resistance and easier bleachability. In carrying out my process, the raw cellulosic material is initially cooked in the usual acid sulphite liquors or in acid sulphite liquors in which chemicals such as sodium sulphate, sodium bisulphite, borax, or the like, undergo progressive metathetical reaction with sulphurous acid to produce sodium bisulphite. This initial cooking operation, however, is carried short of complete fiber liberation, whereupon the cellulosic material is then cooked in a solution of sulphurous acid containing little, if any, SO<sub>2</sub> in combined condition. The second cooking operation may be carried out at lower temperature than the initial cooking operation, for under such lower temperature conditions a sulphur-

ous acid solution containing little, if any, combined SO<sub>2</sub>, is more reactive and more selective in its action upon ligneous constituents in the cellulosic material than the usual acid sulphite liquor. The improved qualities of the resulting product over the usual sulphite pulp may be attributed to the greater hydrolysis of fiber occurring during the usual acid sulphite cook under the progressively increasing temperatures employed to compensate for the removal of free SO<sub>2</sub> from the cooking liquor.

The following specific example of procedure will serve to illustrate conditions under which the process of the present invention may be practised to produce a pulp having markedly better characteristics than the usual sulphite pulp. Spruce or other wood chips are initially cooked while confined in a digester in an acid sulphite liquor containing a substantial proportion of combined SO<sub>2</sub>. The acid sulphite liquor may be of the sodium base or the usual calcium base type, and contain 1% SO<sub>2</sub> combined in the form of sulphite, and 5% SO<sub>2</sub> in free condition.

When a sodium base is employed, it may be preferable to dissolve sufficient sodium base chemical in the liquor to produce a much higher combined SO<sub>2</sub> concentration therein than that of the less soluble calcium base, for instance 3% to 4%, as a more rapid and uniform penetration of the wood by combined SO<sub>2</sub> is ensured. Such higher combined SO<sub>2</sub> concentration permits higher temperature of cooking, as the combined SO<sub>2</sub> in the chips retards hydrolyzing action on the fibers by the free SO<sub>2</sub>. The temperature of cooking in an acid sulphite liquor containing 1% combined SO<sub>2</sub> and 5% free SO<sub>2</sub> should not be higher than 300° F., a temperature of 275° F. preferably being employed, but when an acid sulphite cooking liquor containing, say, 4% combined and 4% free SO<sub>2</sub> is employed, cooking may be carried out at 300° to 325° F., and these higher temperatures may be reached more quickly without danger of a non-uniform action and injury to the fibers. After the chips and liquor have been brought to maximum cooking temperature, such temperature may be maintained for from two to 100

- four hours, depending upon the composition of the particular liquor employed and the maximum temperature of cooking. At the end of this period, the chips are lighter in color than they were originally, but they are still hard because they contain considerable non-fibrous cementitious material, and hence cannot be reduced to pulp unless they are subjected to a severe grinding operation, such as practiced in making ground-wood pulp. The acid liquor is of light color and contains a large proportion of unspent chemical, so that it may be separated, as by draining, from the cooked chips and again used for the cooking of raw wood, additional  $\text{SO}_2$  being dissolved therein, if desired, to compensate for such loss of free  $\text{SO}_2$  as took place during cooking and separation of the cooked chips. In order to minimize the loss of free  $\text{SO}_2$  from the acid cooking liquor, it may be separated from the chips under pressure by pumping it from the confined charge in the digester to another closed digester in which the pulping of other raw wood is to be effected.
- The cooked chips, while still hot and confined in the digester, may be treated with the second cooking liquor consisting of a solution of practically only sulphurous acid, but it is preferable to wash them before adding such cooking liquor to remove substantially all the combined  $\text{SO}_2$  associated therewith after cooking. The sulphurous acid solution employed may contain 3% to 6%  $\text{SO}_2$ , it being preferable to employ liquors of such free  $\text{SO}_2$ , as an excessive period of time is required for completing fiber liberation in more dilute solutions. When using a liquor containing, say, 5% free  $\text{SO}_2$ , cooking of the chips may be carried out at a maximum temperature of 250° F. In order to avoid pressures above 75 to 80 pounds, free  $\text{SO}_2$  may be released from the liquor as cooking proceeds, the released gas being recovered in suitable systems, as ordinarily. If cooking is effected at a temperature of 250° F. for about three to five hours, the chips will be completely pulped, so that the digester contents may then be blown into a pit, where the pulp may be drained or washed free of cooking liquor. The free  $\text{SO}_2$  arising from the pit during the blowing of the digester may be recovered for use in the production of fresh acid liquor, and the separated spent liquor may be mixed with spent liquor resulting from the initial cooking step, when recovery of their valuable constituents is practiced, as for instance when a sodium base cooking liquor is employed in the initial cooking step.
- A pulp produced as hereinbefore described is of high strength and tear resistance and has a high cooking stain value, indicating easy bleachability. I present herein a table showing certain characteristics of a pulp produced as hereinbefore described, and the

usual commercial sulphite pulp produced from spruce:

|               | Product resulting from the process of the present invention | Usual commercial sulphite pulp | 70 |
|---------------|-------------------------------------------------------------|--------------------------------|----|
| Strength      | 150                                                         | 125                            | 80 |
| Tear          | 180                                                         | 150                            | 85 |
| Cooking stain | 120                                                         | 100                            | 90 |

The cooking stain value of 120 indicates that the pulp resulting from the process herein described will require only about 8% calcium hypochlorite bleach to be converted into a white product, whereas the sulphite pulp having a cooking stain of 100 will consume about 15% of such bleach in acquiring the same degree of whiteness.

My process may be practised in a period of time not in excess of the cooking period of the usual acid sulphite process. Were it attempted in such a period of time to produce by the usual acid sulphite process a product having the easy bleachability of the product resulting from my process, it would be necessary to complete fiber liberation at such high temperatures as would cause serious degredation of cellulose and a marked lowering of the strength of the product. On the other hand, were it attempted to produce pulp by cooking in sulphurous acid solutions alone, it would be necessary to cook for exceedingly long periods of time and at a temperature of about 220° F., or lower, owing to the severe hydrolysis of cellulose and injury to the fibers taking place if fiber liberation is hastened by raising the temperature of the cooking liquor. Even when fiber liberation is effected at comparatively low temperature by cooking in a liquor consisting of only sulphurous acid solution, the resulting pulp is so dark that it requires an excessive amount of bleaching agent and undergoes such marked degradation during bleaching as to be of little value for papermaking or other purposes. Apparently the combined  $\text{SO}_2$  content of the usual acid sulphite liquor reacts upon encrustations of the wood in a different way than a sulphurous acid solution alone, this being borne out by the fact that after wood has been cooked with a sulphurous acid solution alone, it cannot readily be converted into fiber by the usual acid sulphite cook. Evidently a sulphurous acid solution causes a resinification or polymerization of certain constituents present in the raw wood to produce reaction products difficultly soluble in the usual acid sulphite liquors, even under high temperature and pressure conditions. By first cooking the wood in an acid sulphite liquor containing combined  $\text{SO}_2$ , for instance the usual acid sulphite liquor, the production of such undesirable reaction products is evidently avoided, so that the fibers of the cooked chips may be readily liberated when fiber liberation is 130

completed in a sulphurous acid solution containing little, if any, combined  $\text{SO}_2$  to produce a finished product having the highly desirable characteristics hereinbefore noted.

- 5 1. I claim:
1. A process which comprises cooking raw cellulosic material short of fiber liberation in an acid sulphite liquor containing at least about 1% combined  $\text{SO}_2$  and then completing fiber liberation at lower temperature in a liquor containing substantially only free  $\text{SO}_2$ .
  2. A process which comprises cooking raw cellulosic material short of fiber liberation in a sulphurous acid solution of a sulphite, separating the liquor from the cooked material, and then cooking the material at lower temperatures in a solution of substantially only sulphurous acid until fiber liberation is complete.
  3. A process which comprises cooking raw cellulosic material short of fiber liberation in an acid sulphite liquor, separating the liquor from the cooked material, washing the material, and cooking the material at lower temperature to complete fiber liberation in a solution of substantially only sulphurous acid.
  4. A process which comprises cooking raw cellulosic material short of fiber liberation in an acid sulphite solution containing at least 1% combined  $\text{SO}_2$  and at temperatures above 250° F., separating the liquor from the cooked material, and then cooking the material to complete fiber liberation in an acid liquor containing less than 1% combined  $\text{SO}_2$  and more than 3% free  $\text{SO}_2$  and at temperatures below 250° F.
  5. A process of fiber liberation which comprises cooking chipped wood in an acid sulphite liquor sufficiently short of fiber liberation so that it contains considerable non-fibrous cementitious material, and then cooking at lower temperature in a solution of substantially only sulphurous acid to complete fiber liberation into a pulp.

In testimony whereof I have affixed my signature.

GEORGE A. RICHTER.